

# UNITED STATES PATENT OFFICE.

CLINTON EMERSON DOLBEAR, OF BOSTON, MASSACHUSETTS, ASSIGNOR TO AMERICAN MINING AND METAL EXTRACTION COMPANY, OF BOSTON, MASSACHUSETTS.

## ELECTROLYTICALLY TREATING ORES.

SPECIFICATION forming part of Letters Patent No. 709,817, dated September 23, 1902.

Application filed June 3, 1901. Serial No. 62,869. (No specimens.)

*To all whom it may concern:*

Be it known that I, CLINTON EMERSON DOLBEAR, a citizen of the United States, and a resident of Boston, in the county of Suffolk and 5 State of Massachusetts, have invented certain new and useful Improvements in Electrolytically Treating Ores, of which the following is a specification.

My invention relates to a new and improved 10 method of producing from raw ores metallic copper or other metals by electrolysis in the wet way.

To carry out my invention, I take a body 15 of the metal-bearing ore that is soluble in a dissolved nitrate or in nitric acid, crush it, and subject it to the action of a nitrate in solution or to nitric acid mixed with sulfuric acid. The object of the nitrate or nitric acid is to furnish the nitric acid radical in quantities sufficient to accomplish the necessary 20 chemical changes. An excess of nitric acid will not interfere with the working of the process. The sulfuric acid will not of itself attack the ores if it be in the state of a sulfid 25 or metallic copper; but in the presence of the nitric acid radical it will do so. If a nitrate be used—for instance, Chile niter, (sodium nitrate)—the sulfuric acid takes the sodium from the nitrate, liberates the nitric acid radical, 30 which in its turn will attack the sulfid, dissolving the base. The sulfuric acid takes the metal from the nitric acid radical, forming 35 the sulfate. During this process the nitric acid loses oxygen, forming nitric oxid, which under usual conditions will rise to the surface and be lost.

In the bath at the bottom of the electrolytic vat I use an insoluble anode—such, for instance, as carbon—though I may use as 40 anodes gold or platinum or any metal that is insoluble in the acids forming the liquid of the bath. The composition of the cathode will depend upon the metal to be plated out of the bath. For instance, if the metal to be 45 plated out is zinc the cathode will be zinc, &c. The anode and the cathode may, if more con-

venient, be placed vertically in the bath, or the anode may be suspended above the cathode.

When current is flowing, the positive terminal will liberate oxygen, which passing 50 through the solution oxidizes the nitric oxid back to nitric acid. This is then in a condition to take up more metal, react with the sulfuric acid, and again go through the process just described. The current, of course, at 55 the same time plates the metal onto the cathode, thereby in one operation giving the desired metal from the raw ore.

The sulfuric acid in combination with the nitric acid radical, whether the same is derived 60 from a nitrate or from nitric acid directly, serves two purposes: first, as a reagent to decompose the nitrate, as stated above, and, second, to assure a reguline deposit of the metal instead of a powdered deposit 65 of the metal, as when a nitrate or nitric acid alone is employed.

Having thus fully described my method, what I claim is—

1. The method of reducing metals from 70 their ores, which consists in dissolving the crushed ores in a nitrate of the suitable metal, adding to the mixture thus formed sulfuric acid, and subjecting the solution to the action of an electric current, whereby the metal 75 is plated out of the solution, substantially as described.

2. The method of reducing metals from 80 their ores, which consists in dissolving the crushed ore in a compound containing a nitric acid radical, adding to the mixture sulfuric acid, and subjecting the resultant compound to the action of an electric current, substantially as described.

Signed at New York, in the county of New 85 York and State of New York, this 18th day of May, A. D. 1901.

CLINTON EMERSON DOLBEAR.

Witnesses:

ALBERT STETSON,  
M. BUTLER.